

July 8, 1958

F. J. BINGLEY

2,842,697

BEAM-INTERCEPTING STRUCTURE FOR CATHODE RAY TUBE

Filed Dec. 7, 1955



FIG. 1.

FIG. 3.



**BEAM-INTERCEPTING STRUCTURE FOR  
CATHODE RAY TUBE**

Frank J. Bingley, Meadowbrook, Pa., assignor to Philco Corporation, Philadelphia, Pa., a corporation of Pennsylvania

Application December 7, 1955, Serial No. 551,648

28 Claims. (Cl. 313—92)

This invention relates to improvements in cathode ray tubes and especially to improved screens for cathode ray tubes used to reproduce scenes televised in colors.

There are systems for the reception of color television signals which employ a cathode ray tube having an image forming, beam-intercepting structure constituted in part of a screen having a plurality of sets of parallel strips of phosphor materials. Each of the sets of strips emits light of a particular color when bombarded by an electron beam. An electron beam, whose intensity is modulated by signals representative of the colors of the scanned elements of a televised scene, is caused to scan said structure in a manner such that, at a time when it is modulated in intensity by a signal representative of, say the red colored elements of the scene, it will impinge only on a phosphor strip emissive of red. An indexing system for coordinating the intensity modulation of the beam with its position on the beam-intercepting screen may be employed so that the colors of the reproduced image are faithful to those of the original televised scene.

If the phosphor strips are disposed contiguous to one another, the area of impingement of the beam, having a finite width, may overlap two adjacent strips. Consequently the red emissive phosphor strip, for example, may be impinged upon by the beam not only during the intervals when the beam is modulated in intensity by signals corresponding to the red color of the scanned element of the televised scene, but also during intervals when it is modulated by blue or green representative signals.

Furthermore, even if the width of the area of impingement of the beam is very small, the faithful rendition of colors is extremely difficult to achieve since there are generally non-linearities in the performance of the beam deflection circuits and components, irregularities in the geometrical disposition of the elements of the beam-intercepting structure, and other practical problems which make exact coordination of beam position and beam modulation very difficult to achieve. An indexing system is extremely helpful in coordinating the modulation of the beam intensity with the position thereof, but even it may be subject to aberrations and inherent limitations which prevent it from being completely effective. As a result of the fact that, in practice, coordination of the beam modulation and position is not always perfectly achieved, the purity of the colors reproduced is adversely affected.

To a certain extent deficiencies in the rendition of colors due to the various factors mentioned above may be overcome by making the individual phosphor strips narrower and spacing them from one another instead of disposing them contiguous to one another so that the scanning beam is less likely to overlap any two adjacent ones of the phosphor strips. The space between any two adjacent phosphor strips also helps to prevent the production of light of any color in the intervals in which

the beam intensity is undergoing a transition from modulations by signals corresponding to the intensity of one color of a televised scene to modulation by signals corresponding to the intensity of a different color. In making the strips narrower and spacing them from one another it becomes possible to increase the brightness of the reproduced image since the scanning beam spot size may be made larger, provided, of course, that it is not wider than the total width of a phosphor strip and the spaces adjacent it on either side. The use of larger beam spots also tends to simplify display tube construction and reduce the costs thereof.

An electron-permeable, light-reflecting, and electrically conductive material is often deposited on the rear (facing the electron-gun) surface of the phosphor strips in order to increase further the brightness of a screen so constructed. This layer increases the brightness of the reproduced image by reflecting back toward the viewer light initially emitted from the fluorescent beam "spot" toward the rear of the tube. It also assists in preventing damage caused by the impact on the phosphor screen of ions which have a much greater mass than the electrons. It is also of use in establishing a desired potential on the rear surface of the phosphor strips.

While the addition of the light-reflecting layer increases brightness, it also introduces some unwanted effects. In addition to reflecting toward the viewer light from the spot emitted in a backward direction, it unfortunately also reflects back to the observer ambient light striking it. For example, if there is a source of illumination in the viewing area, some of its rays will fall on the portions of the light reflecting layer situated in the spaces between the phosphor strips and a mirror image of the source can be seen by the viewer. If daylight enters the viewing area the colored image will be somewhat obscured by the glare from the reflective coating and the colors of the image on the display tube will be desaturated to a certain extent.

Another disadvantage of spaced phosphor strips backed by a layer of light-reflecting material is that the adverse effects of halation are multiplied. Halation occurs because, as the phosphor strips emissive of the various colors are caused to emit light by the electron beam impinging thereupon, the light from the red phosphor strip, for example, will be reflected by the front internal surface of the glass faceplate of the tube back toward phosphor strips emissive of green and blue light, thereby causing the latter colors to be desaturated. Halation may also cause fuzziness in the reproduction of sharp transitions from one color to another in the reproduced image.

It is therefore an object of the present invention to provide systems for improving the quality of luminous images produced by certain types of cathode ray tubes.

Another object of the invention is to provide a screen structure for improving the color fidelity of images reproduced by certain types of color television display tubes.

In the manufacture of the beam-intercepting structures of display tubes such as those previously described, the sets of phosphor strips are frequently deposited upon the inner surface of the faceplate of the cathode ray tube by photographic means. Formerly, in order to maintain color purity, it was imperative to lay down the phosphor strips on the inner surface of the faceplate so that the width of each strip was essentially uniform throughout its entire length. The attainment of this objective is difficult because the particles of the respective phosphor materials used for the strips have different average sizes. The strips of phosphor materials whose particles are relatively large generally have edges whose contour is characterized by large variations, whereas the strips

composed of relatively small phosphor particles tend to have edges whose contour is characterized by relatively small variations. In the present state of the art phosphors emissive of the colors desired cannot be obtained which all have uniformly dimensioned particles of the desired fineness.

Accordingly it is another object of the invention to provide a system for manufacturing beam-intercepting structures of cathode ray tubes of the type described in which the edges of all the phosphor strips are made so that their contour is subject to only very small variations.

It is a further object of the invention to provide a method for manufacturing fluorescent screens in cathode ray tubes of the type desired in which the visible or effective width of the fluorescent strips is maintained uniform despite variations in the particle sizes of the particular fluorescent materials used therein.

Previously also, in the manufacture of screens having spaced phosphor strips some of the phosphor materials inadvertently became lodged in the spaces between adjacent ones of the phosphor strips. Consequently, when the beam traversed these spaces, light of one or more colors was emitted with a resulting loss of color fidelity in the image. It also happened in the manufacture of such screens that, because of inaccuracies in the successive steps of laying down the different sets of phosphor strips, the strips were not displaced laterally from one another according to the specifications. This adversely affected the desired coordination between the beam position and the modulation thereof, with a concomitant loss of color purity. In cases of extreme misplacement of the strips, some particles of the phosphor material of one strip overlapped those of another set so that, toward the edges of the strips, a mixture of colors was produced, with a resulting loss of color purity.

Another object of the invention is to overcome the adverse effects of misplaced phosphor particles on the color quality of the reproduced image.

Still another object of the invention is to simplify the fabrication of such screens by reducing the precision required in depositing the strips in successive steps.

In cathode ray tubes of the type described it is customary to decrease the efficiencies of the naturally more efficient phosphor materials emissive of green and blue light, for example, so as to equalize the light output therefrom with respect to the light output from the less efficient phosphors such as the red phosphor. This procedure naturally results in a reduced efficiency of light output with respect to electrical input to the display tube for a given area of phosphor material.

It is, accordingly, another object of the invention to preserve the advantages of using phosphors which are naturally more efficient while compensating for the phosphors which are less efficient in order to achieve greater image brightness and proper color balance.

These objects, as well as others which will appear, are achieved according to my invention by an improved beam-intercepting structure for cathode ray tubes of the type described, in which a plurality of substantially opaque and non-reflecting "guard" elements are deposited in a predetermined pattern on an appropriate transparent substrate and a plurality of electron-sensitive elements are deposited in a predetermined pattern in the spaces between the opaque and non-reflecting elements. In accordance with one form of the invention as used in color television display apparatus, a plurality of opaque, non-reflecting and elongated elements are deposited on a transparent substrate in a definite pattern and a plurality of elongated phosphor elements which emit light of selected colors in response to electrons impinging thereupon are deposited in the spaces between, and in contact with, the adjacent opaque elements. Preferably, the phosphor elements are so deposited that they overlap on the rear surfaces of the opaque elements. This helps to insure that

the spaces between the guard elements are completely filled by the phosphor elements, yet permits the latter to be deposited with less precision than has heretofore been customary. If an electron-permeable and light-reflecting layer is deposited on the rear surfaces of the phosphor strips and the opaque elements, ambient light falling on the face of the tube will not be reflected back into the observer's line of vision from those portions of the reflective layer situated between the phosphor strips. Halation is also reduced because a considerable portion of the light reflected back onto the screen from the front internal surface of the faceplate is absorbed by the opaque and non-reflective elements.

In another form of the invention, the disparities in the efficiencies of the phosphor materials of the several sets of phosphor strips are equalized by making the widths of the strips of each set vary inversely with the relative efficiency of the phosphor material of which it is composed. Thus, the width of a relatively inefficient phosphor strip, such as the red emissive strip for example, is made large with respect to the width of a relatively efficient phosphor strip such as the green emissive strip. In order to permit the beam intensity to be modulated at a single frequency, the center-to-center distance between any two adjacent phosphor strips, regardless of their width, may be made equal. In some cases, however, it may be desirable to vary the center-to-center distance between adjacent phosphor strips because of other considerations which are not pertinent to the present invention.

In accordance with still another form of the invention an effective method is provided for expediting the production of improved screen structures with a concomitant relaxation of some of the manufacturing tolerances required therein. This system involves the process of first depositing the opaque and non-reflective elements on one surface of an appropriate transparent substrate, and next depositing each of the sets of phosphor strips in turn in the spaces between the opaque strips. Even if each deposited phosphor strip overlaps somewhat on the rear surfaces of the adjacent opaque strips because it is wider than the space therefor, there is no loss of uniformity of the visible width of the phosphor strips or loss of color purity since the opaque strips block light from those portions of the phosphor strips which do overlap and prevent it from reaching the viewer. Thus the phosphor strip deposition process can be performed with less precision than heretofore has been required.

It has previously been stated with respect to previous types of screen structures that the particle sizes of the various phosphors employed are relatively large and thus the edges of the phosphor strips have contours which are subject to rather large variations. In one particularly advantageous form of our invention the particle size of the material of which the opaque guard strips are constituted is very fine in comparison with the particle size of the phosphors. If the guard strips are laid down first, and the phosphor strips next, it is the edges of the guard strips which define the visible edges of the phosphor strips contiguous therewith. Since the material of the guard strips is very fine, their edges have contours which are marked by relatively small variations so that the width of each one can be made very uniform. Thus the visible edges of the phosphor strips defined thereby have contours marked by relatively small variations, and the visible or effective width of each of the phosphor strips is rendered more uniform so that light emitted therefrom is confined with greater precision than has hitherto been possible.

Figure 1 is a sectional perspective view of one form of beam-intercepting structure in accordance with my invention;

Figure 2 is a sectional plan view of the structure shown in Figure 1; and

Figure 3 is a sectional plan view of another form of screen structure in accordance with the invention.

Referring to Figure 1, a beam-intercepting structure for a cathode ray tube used to reproduce images of televised scenes in color is shown. It consists of a transparent substrate 20 which may be the faceplate of the cathode ray tube, for example, or an essentially planar transparent member mounted in proximity thereto. Deposited on the inner surface of the substrate 20 are phosphor strips 21, 22, and 23 which respectively emit green, red and blue light in response to the impingement thereupon of an electron beam (not shown). The phosphor strips 21, 22 and 23 are disposed in recurrent sequence across the screen.

Between the phosphor strips, strips 27 of a substantially opaque and non-reflective material are deposited in accordance with the present invention. The material of the strips 27 may be comprised of ferrous oxide which has been flowed onto the faceplate in the form of a slurry as will be explained below, or may be of graphite. These materials are recited solely as examples which have proved effective in making a screen structure according to the invention. It is preferable that the material be substantially non-reflective but in some cases the material may reflect light of low visibility, as for example, the characteristic dark red of ferrous oxide which may have other desirable properties in addition to good opacity and substantial non-reflectivity.

On the rear surface of the strips 21, 22 and 23 and the strips 27 a conventional electron-permeable and light-reflecting layer 26 is deposited. This layer 26, which may be of aluminum for example, increases the brightness of the reproduced image by reflecting toward the observer those rays of light emitted in the direction of the electron gun from the point where the electron beam impinges on the phosphor strips.

On the rear surface of the layer 26 and coincident with the strips 21, for example, a number of indexing strips 28 may be deposited which may be composed of a material such as MgO, for example, which has a secondary emission ratio different from that of the layer 26, or may be composed of a light emissive phosphor. Indexing signals in the form of a secondary electron current or light variations, as the case may be, are generated in response to the scanning of the electron beam thereupon. These signals may be used in an indexing system (not shown) for coordinating the beam position with the intensity modulation thereof.

The strips 21, 22 and 23 are separated by strips 27 of an opaque and non-reflective material for a number of reasons. The strips 27 assist in preventing the simultaneous impingement of the electron beam upon two adjacent phosphor strips. The strips 27, being opaque and non-reflective, also prevent ambient light from the viewing area from being reflected back to the viewer by the reflective layer 26. This is more readily apparent from inspection of Figure 2 wherein the beam-intercepting structure 19 is shown in a plan and sectional view. Parts in Figure 2 similar to those of Figure 1 are similarly numbered. A ray of ambient light 36 is seen passing through the substrate 20 and striking one of the opaque strips 27. Were the strip 27 on which it falls absent, the ray 36 would be reflected back to the viewer by a portion of the reflecting layer 26. Since the rays of ambient light are largely absorbed by the strips 27 on which they fall, the saturation of the colors of the image as viewed by an observer is improved since they are not diluted by reflected ambient light.

Fig. 2 also depicts how the opaque strips 27 serve to reduce the amount of halation caused by the impingement of ambient light on the novel screen. Another ray 39 of ambient light is reflected from a point 31 adjacent one of the blue color emissive strips 26 in response to the ray 30 incident thereupon onto the front internal surface 35 of the faceplate 20 whence part 33 of it is

once again reflected back onto one of the strips 27 where it is absorbed. Were it not for the presence of the latter strip 27, it would be reflected once again toward the observer by the reflective coating 26.

Fig. 2 also illustrates how the strips 27 assist in reducing the halation which arise as a result of the light emitted from the point where the beam impinges upon the phosphor strips. The electron beam illustrated diagrammatically by the dashed line 40 is scanning the phosphor strips and passes through the electron-permeable layer 26 causing that portion of the blue emissive strip 22 through which it passes to emit light of that color. Most of the blue light rays 42 and 43 pass through the substrate 20 and out to the viewer, but part of the

ray 42 is reflected back onto, and absorbed by, one of the opaque strips 27. The ray 44 from the spot is reflected by the front internal surface 35 back onto the green emissive phosphor 21 at point 48 where at least part of it is again reflected as indicated by the rays emanating from that point. A ray 45 from the luminous spot at point 41 is also reflected in part from internal surface 35 back onto one of the opaque strips 27 where it is absorbed. It is seen that, absent the strips 27 between the phosphor strips, the color purity of the image produced would be subject to considerable deterioration because of the desaturating effect of the halation effects arising from the reflection of the blue light of the spot, onto the adjacent green and red emissive phosphor strips, for example.

Figure 3 illustrates another form of the invention in which the opaque strips 27' intermediate the phosphor strips are of varying width thus masking off part of the phosphor strips from the view of the observer and causing the visible width of the several phosphor strips to differ.

These differences are introduced for the express purpose of compensating for the differences in the efficiencies of the various phosphors employed. The best phosphor materials presently known, which emit red in response to the impingement of electrons thereupon, have a much lower efficiency than the available blue and green light-emissive phosphors. It has been common practice heretofore to adulterate or dilute deliberately the green and blue phosphors so that their effective efficiencies are lowered to correspond to the efficiency of the red emissive phosphors. This obviously reduces the total light output of the image and thereby adversely affects the visibility thereof in the presence of ambient light.

By employing the form of my invention shown in Fig. 3, the maximum natural efficiency ratios of the available phosphor materials emissive of red, blue and green light may be exploited without affecting the balance of colors as viewed by an observer. In this form of the invention the opaque strips may be uniformly wide and the phosphor strips may be of different widths, or both the opaque strips and the phosphor strips may be of different widths. In the particular embodiment shown in Fig. 3 the opaque strips 27' and the phosphor strips 21', 22', and 23' both have different widths. The widths of the opaque strips optionally may be selected so as to achieve a substantially uniform center-to-center spacing  $x$  between any two adjacent phosphor strips so that the beam intensity may be modulated at a single frequency. Thus, for example, the distance  $x$  may be made equal to the corresponding distance  $y$  of Fig. 2. If the center-to-center distance between the phosphor strips is made to vary the beam intensity would be modulated by a signal wave having a complex frequency. In certain other applications the width of the respective phosphor strips may be adjusted arbitrarily to over-emphasize one or more of the colors of the reproduced image or display.

To improve the reproduction of the colored image for the reasons stated previously it is only necessary that the opaque elements 27' be located between adjacent ones 75 of the color emissive phosphor strips. As seen in Fig. 3,

however, the phosphor strips are located not just between the opaque elements 27' but may also overlap them to some extent on their rear surfaces. While the deposition of the phosphor strips in the manner shown in Fig. 3 may appear somewhat wasteful of phosphor material, this possible disadvantage is greatly outweighed by the resultant simplification in the process of manufacturing such structures and the considerable improvement in screen structures provided thereby, which makes possible the reproduction of superior colored images. These advantages will become clearer from the following explanation of some of the factors involved in the manufacture of such tubes.

Previously each set of phosphor strips was deposited upon the substrate 20 by the use of photographic techniques involving the projection of a grill of vertical lines onto a layer of a photo-sensitive material deposited on the inner surface of the faceplate of such a tube. After exposure the photo-sensitive layer was covered with one of the phosphor materials and then the inner surface of the faceplate was washed. Those portions of the photo-sensitive layer which had been exposed to light became hardened and the phosphor material adhered closely thereto, whereas the unexposed portions remained relatively soft so that they, and the particles of the phosphor material deposited thereupon, were washed away. This process is explained in more detail in the co-pending application of P. D. Payne, Jr., Serial No. 376,345, filed August 25, 1953.

The other sets of phosphor strips were deposited in a similar manner, i. e., other grills for the respective sets of phosphor strips were projected upon photo-sensitive materials on the screen and the phosphor materials were deposited in the same fashion. The grills had to be precisely placed so as to fulfill the requirements of extremely precise spacing between the strips to yield a tube capable of reproducing good color images.

In accordance with the present invention, the beam-intercepting structure of such tubes are preferably made by first depositing the opaque elements on the substrate, and then depositing thereupon the electron sensitive phosphor elements whose edges visible to the viewer are defined by the edges of the opaque elements. This has several advantages over former methods, among which are: (1) the positioning of the respective grills after the deposition of each set of phosphor strips is not so critical since, if the phosphor strips are not displaced from one another exactly as specified, they will overlap on the backs of the adjacent opaque elements to a certain extent. However, since the latter are opaque, those portions that do overlap will not be visible to the observer; (2) the visible width of the phosphor strips may be made more uniform. This is due to the fact that the opaque strips may be composed of particles which are much finer and more nearly homogeneous than those of available phosphor strips. Therefore the edges of the opaque strips may have a contour subject to only small variations. Thus the visible edges of the phosphor strips are defined by the more invariant edges of the opaque strips and the effective widths of the phosphor strips are thereby made more uniform, (3) the possibility that some of the phosphors deposited in subsequent processing steps may become lodged in the spaces between adjacent phosphor strips, causing color contamination, is eliminated since the opaque elements are deposited first. Even if some phosphor particles in later steps inadvertently adhere to the rear surfaces of the opaque elements, no color contamination will be caused since the light of the color emitted by the phosphor in response to electron impingement will be blocked from the viewer by the opaque elements.

As stated above, a photographic method of depositing the opaque strips and the sets of phosphor strips may be used which accords with the method explained in the Payne application previously referred to. However, it

should be understood that other methods may be used, provided, however, that the opaque elements are deposited first. For example, the process for depositing the elements of the beam-intercepting structure disclosed in the co-pending application of C. H. Pool, Serial No. 333,726, filed January 28, 1953, may be employed. In that application an improved method of laying down some of the screen elements is set forth, in which the elements are deposited not once but twice in order to improve the characteristic responses of those elements to the scanning thereof by an electron beam.

In practice, the fabrication of the beam-intercepting structure according to the principles disclosed herein, has been very successfully achieved by using the following process:

(1) Coat the inner surface of the faceplate with a photo-sensitive material comprising, for example, water, polyvinyl alcohol, and a denatured alcohol such as that designated by the trademark "Solox" manufactured by the Industrial Solvents Division of the Union Carbide and Chemical Company.

(2) Dry the emulsion.

(3) Project the image of a grill on the coated inner surface of the faceplate.

(4) Flow on a slurry of 70 grams unactivated willemite, 80 cc. "Solox," and 60 cc. water.

(5) Dry.

(6) Wash with water.

(7) Dry.

(8) Deposit another layer of the photo-sensitive material mentioned in step number 1.

(9) Dry.

(10) Project grill image again as in step three.

(11) Flow on a slurry of 30 grams  $Fe_2O_3$ , 20 cc. water, and 120 cc. "Solox." This slurry differs from the slurry described in step four and helps to produce the desired width of the opaque lines. (Alternatively, two slurries of  $Fe_2O_3$  may be applied.)

(12) Dry.

(13) Wash with water.

(14) Dry.

(15) Coat faceplate as in steps number 1 and 8.

(16) Dry.

(17) Project the image of another grill corresponding to the position of one of the sets of phosphor strips on the inner surface of the faceplate.

(18) Flow on a slurry comprising water, "Solox" and the phosphor material emissive of the color desired. Repeat steps 5-14 using a slurry of the phosphor desired instead of the  $Fe_2O_3$  called for in step 11.

(19) After the phosphor strips of one color have been deposited, deposit the strips of the other colors in a similar fashion.

(20) Deposit the reflecting layer 26 on the rear surfaces of the phosphor strips and of the intermediate opaque guard lines.

(21) Deposit the indexing strips 28 on the rear surface of the layer 26 by a process similar to the process by which the guard lines and the phosphor strips are deposited.

The invention is also applicable to other forms of display devices for the production of images in color. For example, it is applicable to the conventional so-called "aperture mask" type of color television display tube which comprises a screen containing a plurality of sets of phosphor dots emissive of light in selected colors, said dots being arranged in a number of "triads," i. e., triangular patterns containing three different color emissive phosphor dots displaced equally from one another, a plurality of electron guns for producing a plurality of beams whose respective intensities are modulated to correspond to the intensities of the colors of the elements of the scene televised, and a perforated mask interposed between the electron guns and the phosphors on the screen to assist in assuring that the respective beams

impinge only on the corresponding sets of phosphors. In conventional aperture mask tubes up to ninety percent of the electron beam current may be dissipated by the perforated mask and only ten percent of the electrons emitted from the electron gun actually may impinge upon the phosphor dots. As a result the brightness of the image produced by such a tube is relatively low. By employing a reflective backing on the back surface of the screen of such a tube the intensity of the luminous image may be considerably increased. However, the presence of a reflective material in the interstices between adjacent ones of phosphor dots causes serious desaturation of the image due to reflected ambient light which is the more marked because of the fact that the image actually produced is of very low brightness. The reflective layer also produces a multiplication of halation effects for reasons explained above in connection with Fig. 2.

It is possible, employing the principles of my invention, to expedite the production of phosphor screens of aperture mask tubes by reducing to a certain extent, the precision required in depositing the successive sets of phosphor dots according to the rigid manufacturing tolerances specified therefor.

A tube of the aperture mask type constructed according to the present invention can be made in the following way. First, an opaque and non-reflective material is deposited on an appropriate substrate, such as the inner surface of the faceplate of the tube, or on a separate planar substrate, in a pattern corresponding to the interstices between the phosphor dots of the completed screen. Second, the respective sets of phosphor dots are deposited in the spaces in the deposited pattern of opaque material.

In practice the pattern of opaque material can be deposited in several ways. One way is to project the image of the aperture mask to be built into a particular tube, or the image of a master aperture plate, onto a photo-sensitive layer which has been deposited upon the substrate of the tube under construction. This photo-sensitive layer should have properties such that those portions which are exposed to light are easily removable in a subsequent washing or dissolving process. After exposure of the photo-sensitive layer, an opaque and substantially non-reflecting material such as ferrous oxide is flowed onto the photo-sensitive layer and is dried. Subsequently, the entire screen is washed with water and the exposed portions of the photo-sensitive material, on which rest the particles of the opaque oxide material, are washed away.

Alternatively one can project the image of a negative mask that is one which is opaque where the projected phosphor dots are to fall and which is transparent where the interstices between the phosphor dots are to be located. The photo-sensitive layer deposited upon the substrate in this case has characteristics opposite those employed in the first method, i. e., those portions which are exposed to light become hardened and insoluble in water. After exposure of this photo-sensitive layer, the ferrous oxide is deposited thereupon, dried, and the entire screen is then washed with water, leaving a pattern of opaque material corresponding to the interstices between the locations where the phosphor dots are subsequently to be placed. This photo-sensitive material may be the same as the one used in the manufacture of screens such as shown in Fig. 1, as has previously been explained.

The sets of phosphor dots may then be deposited in successive steps as has been heretofore customary in the manufacture of such tubes. Previously the phosphor dots were laid down by means of appropriate silk-screen processes (or by purely photographic processes) in which a silk-screen mask (or its photographic equivalent) is rotated clockwise by approximately 120° after the first set of dots is laid down and the second set of

dots is deposited. The mask is then rotated 120° counter clockwise with respect to its first position and the third set of dots is deposited. Since the opaque pattern is deposited first it is not necessary that the phosphor dots actually deposited have exactly circular contours or that they have a configuration which is congruous with the spaces in the pattern of opaque areas which has been previously deposited. The phosphor dots may be slightly larger than the spaces in the opaque pattern; in fact they may overlap onto the rear surface of the pattern of opaque areas provided that the overlap is not so great that the phosphor dot material falls into a space in the pattern to which a phosphor dot emissive of a different color is to be located. Thus, even if the precise spacing of the respective sets of dots is not exactly achieved, the pattern of opaque material masks the actual pattern of phosphor dots from the viewer, those portions of the phosphor dots which are not properly aligned being blocked from sight by the opaque material.

If desired, an electron-permeable and light-reflecting layer may be deposited on the rear surfaces of the phosphor strips and of the opaque areas to enhance the brightness of the reproduced image. It is evident that then the pattern of opaque material will prevent ambient light from being reflected back into the eyes of the viewer from those portions of the light-reflecting layer which would normally be located in the interstices between adjacent phosphor dots.

Other types of tubes used for color television reception such as the so-called "Chromatron" described in the January 1954 issue of "Proceedings of the I. R. E." at page 309 may also profit by embodying the principles of my invention as explained herein. The post-deflection focussing tube described in the December 1955 issue of "Radio-Electronics" at page 90 would be improved by the application of the instant invention thereto.

While the invention has been described with reference to screens for cathode ray tubes for the reproduction of televised scenes in color, it should be understood that the advantages of employing screens constructed according to my invention are also to be gained in cathode ray tubes for monochromatic image production so constructed as to include a plurality of strips of white emissive phosphors backed by a layer of aluminum. In tubes having screens so constructed the effects of ambient light and halation can be considerably reduced resulting in the production of a luminous image which is much sharper and which has much better contrast than conventional types.

It will be understood that still other embodiments and applications of apparatus constructed according to the diverse forms of the invention described herein will occur to those skilled in the art. Consequently, I desire the scope of this invention to be limited only by the appended claims.

What I claim is:

1. An electron beam-intercepting structure for a cathode ray tube comprising: a plurality of electron-sensitive elements arranged in a regular pattern, and a substantially opaque and non-reflecting material disposed between said elements.
2. An electron beam-intercepting structure for a cathode ray tube comprising: a plurality of electron-sensitive elements arranged in a regular pattern, and a plurality of substantially opaque and non-reflecting elements disposed in a regular pattern in the interstices between said electron-sensitive elements.
3. An electron beam-intercepting structure for a cathode ray tube comprising: a plurality of phosphor elements arranged in a predetermined pattern, and a plurality of substantially opaque and non-reflecting elements disposed in a predetermined pattern in the interstices between said phosphor elements, each of said opaque elements being disposed contiguous to adjacent ones of said phosphor elements.

4. An electron beam-intercepting structure for a cathode ray tube comprising: a plurality of electron sensitive elements disposed on a substrate in a predetermined pattern, said elements being emissive of light in response to the impingement of electrons thereupon, and a plurality of substantially opaque and non-reflecting elements disposed in a predetermined pattern in the interstices between said electron-sensitive elements, said non-reflecting elements also being disposed in contiguity to said electron-sensitive elements.

5. An electron beam-intercepting structure for a cathode ray tube comprising: a plurality of sets of phosphor elements arranged in a predetermined pattern, each of said sets being emissive of light of a different selected color in response to the impingement of electrons thereupon, and a substantially non-reflecting material intermediate said electron sensitive elements.

6. An electron beam-intercepting structure for a cathode ray tube comprising: a substrate of an essentially transparent material, a plurality of phosphor elements disposed on said substrate in a predetermined pattern, said sets of elements being respectively emissive of light of different selected colors in response to the impingement of electrons thereupon, and a plurality of substantially opaque and non-reflecting elements, each of said opaque elements being disposed intermediate two adjacent ones of said electron sensitive elements.

7. An electron beam-bearing intercepting structure for a cathode ray tube comprising: a plurality of phosphor elements which are emissive of light in response to the impingement of electrons thereupon, a substantially opaque and non-reflecting material intermediate said phosphor elements, and a layer of reflecting material in contact with said phosphor elements and with said opaque elements.

8. The electron beam-intercepting structure according to claim 7 wherein said reflecting material is situated behind said phosphor and opaque elements.

9. An electron beam-intercepting structure for a cathode ray tube comprising: a substrate of an essentially transparent and non-conductive material, a plurality of phosphor elements disposed in a predetermined pattern and in contact with said substrate, said phosphor elements being emissive of light in response to the impingement of electrons thereupon, a plurality of substantially opaque and non-reflecting elements disposed intermediate said phosphor elements and in contact with said substrate, and a layer of a reflecting material disposed in contact with said phosphor and opaque elements.

10. The beam-intercepting structure according to claim 9 wherein said plurality of phosphor elements are emissive of light of different selected colors.

11. An electron beam-intercepting structure for a cathode ray tube comprising: a plurality of sets of elongated phosphor elements disposed in a predetermined pattern, each of said sets being emissive of light of a different selected color in response to the impingement of electrons thereupon, and a plurality of elongated and substantially non-reflecting elements disposed intermediate said phosphor elements.

12. The structure according to claim 11 wherein said non-reflecting elements are contiguous with said phosphor elements.

13. The structure according to claim 12 wherein said non-reflecting elements are also opaque.

14. A beam-intercepting structure for a cathode ray tube for reproducing colored images comprising: a plurality of sets of phosphor strips disposed in a predetermined pattern in contact with the inner surface of the faceplate of said cathode ray tube, said sets of phosphors being respectively emissive of light in selected colors in response to the impingement of electrons thereupon, a plurality of substantially opaque and non-reflecting strips, each of said opaque strips being disposed intermediate two adjacent ones of said phosphor strips and in contact

therewith, and a layer of a reflecting material disposed in contact with said phosphor strips and said opaque strips.

15. A method for constructing a beam-intercepting structure for a cathode ray tube comprising the steps of: depositing a substantially opaque material in a predetermined pattern on a substrate, said deposited pattern including a plurality of interstices, and depositing an electron-sensitive material in said interstices.

16. The method of constructing a beam-intercepting structure according to claim 15 wherein said electron-sensitive material is so deposited in said interstices that it overlaps said opaque material.

17. A method of constructing a beam-intercepting structure for a cathode ray tube comprising the steps of: depositing a substantially opaque and non-reflective material in a predetermined pattern on a substrate, said deposited pattern including a plurality of interstices, and depositing a plurality of different phosphor materials in said interstices so that said phosphor materials overlap the rear surface of said opaque material.

18. A method of making a beam-intercepting structure for a cathode ray tube comprising the steps of: depositing a substantially opaque and non-reflective material so that the front surface thereof makes contact with a substrate, said opaque material being deposited in a predetermined pattern having a plurality of interstices therein, depositing a plurality of sets of elements composed of respectively different electron-sensitive phosphors on the portions of said substrate exposed by said interstices, each of said elements being so deposited as to have a surface which makes contact with a region of the rear surface of said opaque material lying near each of said interstices, and depositing a light-reflecting material on said rear surface of said opaque material and on the rear surfaces of said phosphor elements.

19. A beam-intercepting structure for a cathode ray tube comprising: a substantially opaque and non-reflective material deposited in a regular pattern on a substrate, said pattern including a plurality of interstices, and a plurality of different phosphor materials deposited in said interstices so that said phosphor materials overlap the rear surface of said opaque material.

20. A beam-intercepting structure for a cathode ray tube comprising: a plurality of strips of a substantially opaque and non-reflective material deposited in a regular pattern on a substrate, said pattern including a plurality of interstices, and a plurality of strips composed of respectively different electron-sensitive phosphors on the portions of said substrate exposed by said interstices, each of said strips being so deposited as to make contact with a region of the rear surfaces of said opaque strips near each of said interstices.

21. The structure according to claim 20 and further comprising a light-reflecting material deposited on said rear surfaces of said opaque strips and on the rear surfaces of said phosphor strips.

22. An electron beam-intercepting structure for a cathode ray tube comprising a plurality of mutually spaced strips of opaque material deposited on a substrate and different phosphor material deposited in the spaces between said strips, said spaces having widths which are a function of the respective efficiencies of the phosphor materials deposited therein.

23. An electron beam-intercepting structure for a cathode ray tube comprising a plurality of mutually spaced strips of opaque material deposited on a substrate, and phosphor materials deposited in the spaces between said strips, the phosphor material deposited in certain of said spaces having an efficiency differing from that of those deposited in others of said spaces, the spaces occupied by phosphor material of lower efficiency being wider than those occupied by phosphor material of higher efficiency.

24. The structure according to claim 23 and further

comprising a light-reflecting layer deposited on the rear surfaces of said opaque strips and of said phosphor materials.

25. The structure according to claim 24 wherein said opaque strips have a plurality of different widths.

26. The structure according to claim 25 wherein the center-to-center distance of the phosphor materials deposited in adjacent spaces is substantially the same.

27. A beam-intercepting structure for a cathode ray tube comprising: a substantially opaque and non-reflective material deposited in a regular pattern on a substrate, said pattern including a plurality of interstices, and phosphor material deposited in said interstices in a regular pattern, the particles of said phosphor material being larger than the particles of said opaque material. 10

28. A beam-intercepting structure for a cathode ray 15

tube comprising: a substantially opaque and non-reflective material having particles of a given size deposited in a regular pattern on a substrate, said pattern having a plurality of interstices, and a plurality of sets of phosphor elements deposited in said interstices, said sets of phosphor elements having respective particle sizes substantially larger than said given size.

References Cited in the file of this patent

UNITED STATES PATENTS

|           |           |       |               |
|-----------|-----------|-------|---------------|
| 2,137,118 | Schleede  | ----- | Nov. 15, 1938 |
| 2,388,203 | Zindel    | ----- | Oct. 30, 1945 |
| 2,446,440 | Swedlund  | ----- | Aug. 3, 1948  |
| 2,446,791 | Schroeder | ----- | Aug. 10, 1948 |
| 2,687,360 | Michaels  | ----- | Aug. 24, 1954 |